

# United States Patent

Forbes et al.

[15] 3,637,500

[45] Jan. 25, 1972

[54] **LUBRICATING COMPOSITIONS**

[72] Inventors: **Eric Simon Forbes, Woking; Keith George Allum, Bagshot, both of England**

[73] Assignee: **The British Petroleum Company Limited, London, England**

[22] Filed: **July 17, 1970**

[21] Appl. No.: **55,967**

**Related U.S. Application Data**

[63] Continuation-in-part of Ser. No. 700,022, Jan. 24, 1968, abandoned.

[30] **Foreign Application Priority Data**

Jan. 31, 1967 Great Britain ..... 4,581/67

[52] U.S. Cl. ..... 252/48.6, 252/56 R, 252/57

[51] Int. Cl. ..... C10m 1/42, C01m 1/38

[58] **Field of Search** ..... 252/48.6, 45, 56, 56 S

[56]

**References Cited**

**UNITED STATES PATENTS**

|           |        |                    |            |
|-----------|--------|--------------------|------------|
| 2,110,281 | 3/1938 | Adams et al. ....  | 252/45     |
| 2,744,070 | 5/1956 | Baker et al. ....  | 252/45 X   |
| 3,337,457 | 8/1967 | Fowler et al. .... | 252/56 S X |

**FOREIGN PATENTS OR APPLICATIONS**

1,047,493 11/1966 Great Britain ..... 252/56

*Primary Examiner*—Daniel E. Wyman

*Assistant Examiner*—W. Cannon

*Attorney*—Morgan, Finnegan, Durham & Pine

[57]

**ABSTRACT**

Synthetic ester lubricants and certain organic sulfide load-carrying additives form a synergistic mixture when added to mineral base oils, and there is a marked increase in the load-carrying properties of the base oil.

**12 Claims, No Drawings**

## LUBRICATING COMPOSITIONS

## CROSS-REFERENCE TO RELATED APPLICATION

This application is a continuation-in-part of copending application Ser. No. 700,022, filed Jan. 24, 1968, now abandoned.

This invention relates to improvements in lubricating compositions; in particular it relates to lubricating compositions which comprise synergistic mixtures of additives.

## BACKGROUND OF THE INVENTION

It is generally considered that load-carrying additives may be divided into two classes, namely antiwear and extreme pressure additives. When two lubricated moving surfaces are lightly loaded against each other, they are separated by an elastohydrodynamic oil film: as the load increases so the oil film thickness decreases. When the oil film thickness approaches the dimensions of the surface roughness, it will be penetrated by surface asperities: it is in this region that antiwear additives function by improving the oil film strength and thus reducing intermetallic contact. As the load is increased further, the bulk oil film collapses and antiwear additives are no longer sufficient to protect the surface. Extreme pressure additives function in this region by reacting with the metal surface to form an inorganic iron compound, such as iron sulphide, which prevents welding of the metal surfaces.

It is known to add certain esters to mineral oils to improve their load-carrying capacity (see, for example, the recent United Kingdom Pat. No. 1,047,493).

However, it was quite unexpected to find that the addition of a small proportion of ester to a mineral oil containing a small proportion of a load-carrying additive augmented the additive response and indeed, caused certain additives, which previously showed no load-carrying activity at all, to improve the load-carrying capacity of a mineral base oil to a remarkable degree.

## DESCRIPTION OF THE INVENTION

This invention, therefore, provides an improved lubricating composition based on a mineral base oil and which contains up to 20 percent by weight of an ester and up to 20 percent by weight of a load-carrying additive.

Preferably the ester is a polyester containing two ester linkages per molecule, i.e., a diester. The most preferred diesters are those which are liquids or low melting solids.

Examples of suitable diesters are the compounds of the general formula



wherein R represents a saturated hydrocarbon, i.e., alkylene, group having from 1 to 25 carbon atoms or a phenylene group and A and B are the same or different and represent alkyl

groups, each group containing from 1 to 10 carbon atoms, for example, diethyl sebacate.

Other suitable diesters of Formula I are di-alkyl octadecan-1,18-dioate, di-alkyl-tetracosane-1,24-dioate, di-alkyl phthalate, di-alkyl adipate and di-alkyl sebacate, each of the alkyl groups containing from 1 to 10 carbon atoms.

Preferably the load-carrying additive is an organic disulphide, and the lubricating composition preferably contains 0.1 to 10 percent by weight of the ester and 0.1 to 10 percent by weight of the disulphide.

Examples of suitable disulphides are the compounds of the general formula



15 wherein E and F are the same or different and represent alkyl, cycloalkyl, aryl, alkaryl or aralkyl groups, each of which may possibly be substituted by ester groups, and wherein at least one of E and F contains up to 20 carbon atoms. Preferably E and F are alkyl, cycloalkyl, aryl or alkaryl groups containing 20 up to 10 carbon atoms each.

Suitable disulphides include di-n-butyl disulphide, di-cyclohexyl disulphide, 2,2'-(dicarboethoxy)diethyl disulphide, diphenyl disulphide and dibenzyl disulphide.

The mineral oil used depends on the use to which it is to be put and any lubricating oil can be used.

The lubricating composition according to the invention can also contain, if desired, other additives, for example, dispersants, detergents, viscosity index improvers, oxidation and corrosion inhibitors and pour point depressants. The lubricating compositions according to the invention can be used to lubricate, for example, automotive crankcases and transmission systems.

The invention also relates to a method of operating machinery wherein a lubricating composition based on a mineral base oil and which contains up to 20 percent by weight of an ester and up to 20 percent by weight of a load-carrying additive is used as the lubricant.

## DESCRIPTION OF THE PREFERRED EMBODIMENTS

40 The invention is illustrated in the following table which compares a number of lubricating compositions according to the invention with reference lubricating compositions. In most cases the lubricating composition according to the invention contain equivalent molar quantities of ester and load-carrying additive. Tests on the various compositions were carried out using a Shell Four-Ball Machine.

The antiwear test was carried out under a load of 15 kg.; at a running speed of 1,500 revolutions per minute, and wear scars on the balls were measured after 30, 45 and 60 minutes, respectively.

Using such conditions of light loading and long running times the test measures antiwear, rather than extreme pressure properties of the compositions. E. R. Braithwaite, "Lubrication and Lubricants," Elsevier Publications, 1967, p. 42.

TABLE

| Compound | Concen-<br>tration,<br>weight<br>percent | Base oil            | Anti-wear test,<br>wear scar diameter<br>in m.m. |            |            |
|----------|------------------------------------------|---------------------|--------------------------------------------------|------------|------------|
|          |                                          |                     | 30<br>min.                                       | 45<br>min. | 60<br>min. |
| 1.       |                                          | Liquid<br>paraffin. | .59                                              | .72        | .81        |
| 2.       | Diethyl sebacate                         | 4.775               | do                                               | .60        | .70        |
| 3.       | do                                       | 2.388               | do                                               | .54        | .64        |
| 4.       | do                                       | 1.194               | do                                               | .52        | .66        |
| 5.       | do                                       | 1.114               | do                                               | .55        | .61        |
| 6.       | do                                       | 0.597               | do                                               | .64        | .63        |
| 7.       | do                                       | 0.299               | do                                               | .57        | .63        |
| 8.       | do                                       | 0.286               | do                                               | .53        | .61        |
| 9.       | do                                       | 0.072               | do                                               | .57        | .61        |
| 10.      | Di-n-butyl disulphide                    | 3.296               | do                                               | .78        | .81        |
| 11.      | do                                       | 1.648               | do                                               | .69        | .76        |
| 12.      | do                                       | 0.824               | do                                               | .78        | .89        |
| 13.      | do                                       | 0.412               | do                                               | .82        | .86        |
| 14.      | Diethyl sebacate                         | 4.775               | do                                               | .43        | .45        |
| 15.      | Di-n-butyl disulphide                    | 3.296               | do                                               | .51        | .55        |
|          | Diethyl sebacate                         | 2.388               | do                                               | .51        | .55        |
|          | Di-n-butyl disulphide                    | 1.643               | do                                               | .51        | .55        |

| Compound | Concentration,<br>weight<br>percent                                            | Base oil                                                          | Anti-wear test,<br>wear scar diameter<br>in m.m. |            |            |
|----------|--------------------------------------------------------------------------------|-------------------------------------------------------------------|--------------------------------------------------|------------|------------|
|          |                                                                                |                                                                   | 30<br>min.                                       | 45<br>min. | 60<br>min. |
| 16.      | {Diethyl sebacate<br>Di-n-butyl disulphide                                     | 1.194<br>0.821                                                    | do                                               | .62        | .63        |
| 17.      | {Diethyl sebacate<br>Di-n-butyl disulphide                                     | 0.597<br>0.410                                                    | do                                               | .69        | .71        |
| 18.      | {Diethyl sebacate<br>Di-cyclo-hexyl disulphide                                 | 4.260<br>4.775                                                    | do                                               | .63        | .70        |
| 19.      | {Diethyl sebacate<br>Di-cyclo-hexyl disulphide                                 | 4.260<br>(-S-CH <sub>2</sub> -CH <sub>2</sub> COOEt) <sub>2</sub> | do                                               | .40        | .46        |
| 20.      | {Diethyl sebacate<br>(-S-CH <sub>2</sub> -CH <sub>2</sub> COOEt) <sub>2</sub>  | 2.462<br>1.231                                                    | do                                               | .68        | .75        |
| 21.      | do                                                                             | 1.231                                                             | do                                               | .56        | .64        |
| 22.      | do                                                                             | 0.617                                                             | do                                               | .49        | .55        |
| 23.      | {Diethyl sebacate<br>(-S-CH <sub>2</sub> -CH <sub>2</sub> -COOEt) <sub>2</sub> | 4.775<br>2.462                                                    | do                                               | .50        | .54        |
| 24.      | {Diethyl sebacate<br>(-S-CH <sub>2</sub> -CH <sub>2</sub> -COOEt) <sub>2</sub> | 4.775<br>1.231                                                    | do                                               | .41        | .41        |
| 25.      | {Diethyl sebacate<br>(-S-CH <sub>2</sub> -CH <sub>2</sub> -COOEt) <sub>2</sub> | 4.775<br>0.617                                                    | do                                               | .34        | .37        |
| 26.      | {Diethyl sebacate<br>(-S-CH <sub>2</sub> -CH <sub>2</sub> -COOEt) <sub>2</sub> | 0.597<br>0.617                                                    | do                                               | .45        | .51        |
| 27.      | Di-phenyl disulphide                                                           | 4.037                                                             | do                                               | .44        | .47        |
| 28.      | Diethyl sebacate                                                               | 4.775                                                             | do                                               | .40        | .38        |
| 29.      | Di-phenyl disulphide                                                           | 4.037                                                             | do                                               | .48        | .52        |
| 30.      | Di-phenyl disulphide                                                           | 4.558                                                             | do                                               | .38        | .44        |
| 31.      | Diethyl sebacate                                                               | 4.775                                                             | do                                               | .49        | .49        |
| 32.      | Di-phenyl disulphide                                                           | 4.558                                                             | do                                               | .38        | .44        |
| 33.      | Di-iso-octyl sebacate<br>Di-octyl sebacate                                     | 10.000<br>10.000                                                  | do                                               | .66        | .75        |
| 34.      | Di-iso-octyl sebacate<br>Di-phenyl disulphide                                  | 4.037<br>6.340                                                    | do                                               | .33        | .37        |
| 35.      | Dimethyl octadecan 1-18<br>diolate                                             | 6.340                                                             | do                                               | .552       | .633       |
| 36.      | Dimethyl octadecan 1-18<br>diolate                                             | 6.340                                                             | do                                               | .437       | .451       |
| 37.      | Di-n-butyl disulphide                                                          | 3.296                                                             | do                                               | .455       | .499       |
| 38.      | Dimethyl tetracosane 1-24<br>diolate                                           | 7.890                                                             | do                                               | .597       | .662       |
| 39.      | Dimethyl tetracosane 1-24<br>diolate                                           | 7.890                                                             | do                                               | .437       | .511       |
| 40.      | Dimethyl tetracosane 1-24<br>diolate                                           | 7.890                                                             | do                                               | .455       | .499       |
| 41.      | Di-phenyl disulphide                                                           | 3.296                                                             | do                                               | .496       | .512       |
| 42.      | Dimethyl phthalate                                                             | 3.590                                                             | do                                               | .637       | .712       |
| 43.      | Dimethyl phthalate                                                             | 3.590                                                             | do                                               | .496       | .512       |
| 44.      | Di-n-butyl disulphide                                                          | 3.296                                                             | do                                               | .640       | .720       |
| 45.      | Diethyl adipate                                                                | 3.740                                                             | do                                               | .620       | .649       |
| 46.      | Diethyl adipate                                                                | 3.740                                                             | do                                               | .620       | .650       |
| 47.      | Di-n-butyl disulphide                                                          | 3.296                                                             | do                                               | .578       | .620       |
| 48.      | Di-allyl disulphide                                                            | 2.706                                                             | do                                               | .578       | .620       |
| 49.      | Di-allyl disulphide                                                            | 2.706                                                             | do                                               | .578       | .620       |
| 50.      | Diethyl sebacate                                                               | 4.775                                                             | do                                               | .430       | .480       |
| 51.      | Diethyl sebacate                                                               | 4.775                                                             | do                                               | .430       | .480       |

It can be seen from this table that the addition of an ester to a mineral oil containing a load-carrying additive improves the load-carrying capacity of the composition and that this improvement is obtained at a range of additive concentrations.

It is seen that increasing the amount of ester in the base oil/ester composition can worsen the antiwear result. This is demonstrated by compositions Nos. 2-9 of the table, composition No. 2 being considerably worse than No. 3 and worse than any of the other results.

In composition No. 31 it can be seen that the antiwear performance of the ester plus base oil composition at a 10 percent concentration of ester is worse than that of the base oil alone.

With regard to the disulphide component, di-n-butyl-disulphide, as is shown in compositions Nos. 10-13, leads to considerably worse antiwear performance than the base oil at all concentrations—even though it is known to have extreme pressure properties.

Thus it can be concluded that composition No. 14, for example, has an antiwear performance unexpectedly better than the best diester/base oil composition, and better than the best di-n-butyl disulphide composition. It is unexpected to find this degree of performance because it is not possible to obtain such low antiwear results using any amount of diethyl sebacate or di-n-butyl disulphide by themselves. 60 65

With regard to the other data in the table, it can be seen from compositions Nos. 18, 19, 27 and 28 that the presence of diethyl sebacate can produce an antiwear result when added in conjunction with the disulphide considerably better than that of the organic disulphide by itself. 70

Further unexpected results are shown in compositions Nos. 4, 21 and 26. In No. 4, 1.194 percent weight of diethyl sebacate is used, in No. 21, 1.23 percent weight of 2,2'-(dicarboethoxy)diethyl disulphide is used. As can be seen, the wear scar diameters for the mixture of diester and disulphide at very

nearly equal total concentrations of additives are below the levels attained with the corresponding blends containing either component alone.

In addition it is seen that in compositions Nos. 40 and 41, the blend of diethyl adipate and base oil has worse antiwear performance than the base oil alone, as has the disulphide alone, compositions Nos. 10-13, yet when they are mixed together, they bring about a marked improvement in wear resistance.

We claim:

1. A lubricating composition which comprises
    - i. a mineral oil in major amount;
    - ii. up to 20 percent by weight of a diester of the general formula



wherein R is a saturated alkylene group of from 1 to 25 carbon atoms or a phenylene group; and

A and B, independently, are alkyl of from 1 to 10 carbon atoms; and

iii. up to 20 percent by weight of an organic disulphide load carrying additive, said organic disulphide being of the general formula



wherein E and F, independently, are alkyl, cycloalkyl, aryl, alkaryl, aralkyl and ester-substituted such groups and

wherein at least one of E and F contains from 1 to 20 carbon atoms, the amount of said diester and disulphide in said composition each being in the range of from at least sufficient to impart a marked, synergistic increase in the load carrying properties of said oil to 20 percent by weight.

- ## 2. A lubricating composition which comprises

- i. a mineral oil in major amount;
- ii. from 0.1 to 10 percent by weight of a diester selected from di-alkyloctadecan-1,18-dioate, di-alkyl tetracosane-1,24-dioate, di-alkyl phthalate, di-alkyl adipate or di-alkyl sebacate, each of the alkyl groups containing from 1 to 10 carbon atoms, and
- iii. 0.1 to 10 percent by weight of an organic disulphide selected from di-n-butyl disulphide, di-cyclohexyl disulphide, diphenyl disulphide, dibenzyl disulphide or 2,2-(dicarboethoxy)-diethyl disulphide.
- 3. A composition as defined in claim 2 wherein said diester is diethyl sebacate and said disulphide is di-n-butyl disulphide.
- 4. A composition as defined in claim 2 wherein said diester is diethyl sebacate and said disulphide is di-cyclohexyl disulphide.
- 5. A composition as defined in claim 2 wherein said diester is diethyl sebacate and said disulphide is 2,2-(dicarboethoxy)-diethyl disulphide.
- 6. A composition as defined in claim 2 wherein said diester

- is diethyl sebacate and said disulphide is diphenyl disulphide.
- 7. A composition as defined in claim 2 wherein said diester is di-iso-octyl sebacate and said disulphide is diphenyl disulphide.
- 8. A composition as defined in claim 2 wherein said diester is dimethyl octadecan-1,18-dioate and said disulphide is di-n-butyl disulphide.
- 9. A composition as defined in claim 2 wherein said diester is dimethyl tetracosan-1,24-dioate and said disulphide is di-n-butyl disulphide.
- 10. A composition as defined in claim 2 wherein said diester is dimethyl octadecan-1,18-dioate and said disulphide is diphenyl disulphide.
- 11. A composition as defined in claim 2 wherein said diester is dimethyl phthalate and said disulphide is di-n-butyl disulphide.
- 12. A composition as defined in claim 2 wherein said diester is diethyl adipate and said disulphide is di-n-butyl disulphide.

\* \* \* \* \*